

Nov. 1, 1966

E. H. MAYER ET AL

3,282,685

LOW CARBON STEEL ALLOY FOR VITREOUS ENAMELING

Filed Aug. 8, 1963

3 Sheets-Sheet 1

Fig. 1



INVENTORS

Edward H. Mayer  
BY Hilton N. Rahn  
Evan M. Oliver

Nov. 1, 1966

E. H. MAYER ET AL

3,282,685

LOW CARBON STEEL ALLOY FOR VITREOUS ENAMELING

Filed Aug. 8, 1963

3 Sheets-Sheet 2

EFFECT OF COPPER ON ETCH RATE



Fig. 2

% COPPER

INVENTORS  
BY  
Edward H. Mayer  
Hilton N. Rahn  
Evan M. Oliver

Nov. 1, 1966

E. H. MAYER ET AL

3,282,685

LOW CARBON STEEL ALLOY FOR VITREOUS ENAMELING

Filed Aug. 8, 1963

3 Sheets-Sheet 3

Fig. 3

EFFECT OF TIN ON ETCH RATE



INVENTORS

BY  
Edward H. Mayer  
Hilton N. Rahn  
Evan M. Oliver

# United States Patent Office

3,282,685

Patented Nov. 1, 1966

1

3,282,685

## LOW CARBON STEEL ALLOY FOR VITREOUS ENAMELING

Edward H. Mayer, Hilton N. Rahn, and Evan M. Oliver,  
Bethlehem, Pa., assignors, by mesne assignments, to  
Bethlehem Steel Corporation, a corporation of Delaware

Filed Aug. 8, 1963, Ser. No. 300,849  
2 Claims. (Cl. 75—125)

This invention is directed to a very low carbon vitreous enameling steel having a controlled etching rate as a result of a controlled range of residual alloy content.

In recent years so called "zero carbon" or "special low carbon" steels of approximately the following composition have been widely adopted as a base for vitreous enamel coatings:

|                     | Percent |
|---------------------|---------|
| Carbon, maximum     | .010    |
| Manganese           | .15/.50 |
| Phosphorus, maximum | .010    |
| Sulphur, maximum    | .030    |

The development of these steels eliminated the source of many of the surface defects in the vitreous enamels, and since it was no longer necessary to use a blue ground coat of enamel to cover up the defects originating in the iron base, efforts to develop single-coat, direct-on enameling practices were greatly accelerated.

In the standard two-coat vitreous enameling practice the ground coat contains sufficient cobalt and/or nickel to aid in bonding the enamel to the base metal and the degree of surface roughening of the base metal is not critical. However, with single-coat, direct-on enamels, acid etching of the base metal in controlled amounts and at controlled rates is desirable in order to insure satisfactory bond.

Etching should not be confused with pickling. Pickling and etching are two well known, complementary metallurgical processes that are widely used to condition the surface of ferrous base alloys. Both processes utilize mineral acids, but pickling acid, which is meant to remove accumulated oxide or scale, usually contains an addition agent designed to inhibit the acid attack of the metal proper. In acid etching, where the object is removal of metal, the acid often includes an addition agent designed to accelerate the rate of acid attack on the metal. Although pickling is an extremely complex process it may be considered as a process of using acid to dissolve iron oxide scale whereas in etching the removal of metal is often accompanied by breaking down the acid with the resultant evolution of hydrogen. Technically, pickling is complete when all the scale has been removed. However, etching would immediately commence because even inhibited acid would start to react with the bare metal. Moreover, since the nature of the oxide scale may vary in different locations it is not unusual for these two complementary processes to take place at the same time. However, in the absence of any oxide film or scale there cannot be any pickling, and etching will be the only result of acid attack.

The proper degree of roughening for enameling is often defined in terms of etching to remove a specific weight of metal for a given unit of area (gms./sq. ft.) but there has been no general agreement as to the amount of weight loss which is necessary in order to insure enamel adherence adequate to prevent damage to the enamel coating in normal handling and shipping. Heretofore materials from different producers and also different batches of material from the same producer have varied widely in their susceptibility to acid attack. In a porcelain enameling production line this variation in etching char-

2

acteristics necessitates frequent testing for enamel adherence and modification in the etch tank conditions to compensate for the variation in the base material which in turn has limited the large scale acceptance of direct-on, one-coat enamels in existing enameling lines designed for two-coat enamels. More particularly, it has heretofore been impossible to produce "zero carbon" enameling irons having uniform and predictable etching rates.

The principal object of this invention is to produce an iron base alloy having sufficient adherence for a direct-on, single-coat vitreous enamel to permit substitution into present two-coat enameling lines without observing any special precautions.

Another object of this invention is to provide an iron base material for single-coat, direct-on vitreous enamels which will have a relatively uniform etching rate and eliminate the necessity for control tests on the enameling line.

Another object of this invention is to provide an enameling iron in which the possibility of over-etching is reduced or eliminated.

Another object of this invention is to provide an enameling iron in which the possibility of under-etching is reduced or eliminated and with it the associated problems due to the lack of an adequate bond for a single-coat, direct-on vitreous enamel coating.

Another object is to provide an iron base material for vitreous enameling which will have a predictable etching rate.

Another object is to provide an enameling iron which will have an etching rate (hereinafter more fully defined) of between .14 and .46 gm./sq. ft./min.

Another object is to provide an enameling iron which, when flash coated with nickel and thereafter vitreous enameled, according to standard practices for direct-on enameling, will have an adherence index of not less than approximately 80 when subjected to the standard adherence test prescribed by the Porcelain Enameling Institute.

Another object of this invention is to produce thin sheets of an iron base alloy having good deep drawing characteristics, a predictable etching rate, resistance to sagging at enamel firing temperatures, freedom from enamel defects and sufficient single-coat direct-on enamel adherence to permit normal handling and shipping of the enameled parts without special precautions to avoid failures of the enameled surface.

Although it has been previously recognized that enamel adherence is related to the amount of metal removed by acid etching, the effect of etch rate on said amount is a novel discovery of applicants.

These objects are accomplished in the present invention by maintaining the copper, tin and molybdenum contents of a so-called "zero carbon" enameling iron within certain specifically defined limits, as is more fully set out hereinafter.

In the drawings:

FIG. 1 is a graph wherein the dashed lines depict the extent of the effect of molybdenum on etch rate.

FIG. 2 is a graph wherein the dashed lines depict the extent of the effect of copper on etch rate.

FIG. 3 is a graph wherein the dashed lines depict the extent of the effect of tin on etch rate.

This invention lies in the compositions of an iron base alloy having a range of etching rates which will result in a weight loss of .14/.46 gm./sq. ft./min. when immersed in dilute sulphuric acid (containing 6.5%  $H_2SO_4$  by weight) at a temperature of 158° F. The iron base alloy of this invention when etched at the above rate to remove a minimum of .75 gm./sq. ft., flash coated with nickel,

and direct-on, single-coat enameled, will have a minimum adherence index of not less than approximately 80 when tested by the standard test of the P.E.I. The P.E.I. adherence test is the standard quantitative test for measuring the adherence of vitreous enamel and was developed at the Bureau of Standards. This test involves the systematic deformation of the enameled sheet into a circular die by means of a sphere or rounded plunger. After a suitable interval, adherence is measured electrically by means of a standard series of probes. Experience has shown that an 80 minimum P.E.I. adherence index is sufficient to prevent damaging the enamel coating during normal handling and shipping on a production basis.

It has been hitherto impossible to consistently produce "zero carbon" enameling sheet steels having the desired etch rate and enamel adherence referred to above. We have developed compositions which will consistently have all of said properties. Our invention consists in (a) producing a steel consisting essentially of following compositions by weight:

|                     | Percent   |
|---------------------|-----------|
| Carbon, maximum     | .010      |
| Manganese           | .15/.75   |
| Molybdenum, maximum | .049      |
| Copper              | .014/.060 |
| Tin                 | .001/.030 |
| Iron, balance.      |           |

and (b) adjusting the proportions of molybdenum, copper and tin in accordance with the following formula

$$(.00489/\text{percent Cu}) - (6.605 \times \text{percent Mo}) - (.084 \times \log_{10} \text{percent Sn}) - (.1367) = X$$

where X is a number between .14/.46.

The upper limit of .030% tin is dictated not by etching characteristics or enamel adherence but by the fact that greater amounts of tin increase the susceptibility to hot shortness. The upper limit of .06% on copper is dictated by the fact that greater amounts of copper appear to have an adverse effect on enamel adherence. The upper limit of .049% molybdenum is determined by the minimum etch rate of .14 gm./sq. ft./min.

Under production conditions we prefer to use the following practical limits of composition by weight:

|                 | Percent   |
|-----------------|-----------|
| Carbon, maximum | .010      |
| Manganese       | .15/.75   |
| Molybdenum      | .001/.005 |
| Copper          | .014/.040 |
| Tin             | .001/.005 |

Compositions falling within the above limits will satisfy the formula and produce a sheet steel having good rolling properties which will etch at a rate of .14/.46 gm./sq. ft./min. and have good enamel characteristics but these limits should not be considered as limitations of the invention.

FIGS. 1, 2 and 3 are graphs depicting the effects of molybdenum, copper and tin on etch rate. Although the effect of molybdenum shown on FIG. 1 indicates that this element may be entirely eliminated, parallel situations do not exist for copper and tin as shown on FIGS. 2 and 3. As the copper and tin approach zero the etch rate begins to approach infinity and we have found that as the etch rate exceeds approximately .46 gm./sq. ft./min. difficulties with the enamel are encountered with increasing frequency. These difficulties are in the nature of:

(1) Excessive pickup of nickel during nickel flashing which tends to reduce enamel adherence, and

(2) Accumulation of an etching smut or deposit which requires an additional rinse and/or scrubbing to prevent enamel defects or discolorations.

Table I shows examples of the composition of eight different heats of "zero carbon" enameling steels listed

in the order of increasing etch rate. Steels 4 to 7 are representative of this invention, and steels 1-3 and 8 are illustrative of the composition of steels having etch rates outside the scope of this invention.

TABLE I

|    | C    | Mn  | P    | Mo   | Cu   | Sn   | Etch Rate |
|----|------|-----|------|------|------|------|-----------|
| 10 | .003 | .34 | .009 | .004 | .066 | .005 | .08       |
|    | .004 | .38 | .008 | .015 | .032 | .004 | .11       |
|    | .003 | .32 | .008 | .002 | .050 | .003 | .11       |
|    | .003 | .32 | .008 | .002 | .055 | .003 | .15       |
|    | .004 | .32 | .008 | .005 | .018 | .002 | .30       |
|    | .004 | .31 | .007 | .006 | .015 | .004 | .35       |
|    | .002 | .38 | .014 | .002 | .014 | .002 | .43       |
|    | .002 | .34 | .014 | .002 | .013 | .001 | .49       |

The other elements in this iron base alloy are present in the normal amounts expected in steel sheet intended for enameling and following is a specific example of a steel sheet embodying the invention:

|                | Percent |
|----------------|---------|
| Carbon         | .003    |
| 25 Manganese   | .35     |
| Phosphorus     | .01     |
| Sulphur        | .026    |
| Silicon        | .01     |
| Nickel         | .04     |
| 30 Chromium    | .02     |
| Aluminum       | .005    |
| Nitrogen       | .0025   |
| Copper         | .033    |
| Molybdenum     | .002    |
| 35 Tin         | .004    |
| Iron, balance. |         |

Preferably, we produce this material by making a heat of rimmed steel having a carbon content normal for rimmed steels, e.g. .06/.08% and manganese .15/.75%. We select the raw materials to keep the molybdenum, copper and tin within the limits expressed by the equation and use a clean furnace to avoid picking up these alloys from the refractories. The steel is poured, rolled, decarburized, etc. in the usual manner to produce a soft material free of organic contaminants and iron oxide.

It is well known that the same ferrous material may vary in its susceptibility to etching in different mineral acids (such as nitric, sulphuric, hydrochloric, etc.) as well as in different concentrations of the same acid. It is also known that additives, such as oxidizing agents, or mixtures of acids affect the reaction rate of a particular etchant. The preferred etchant used in this invention is dilute sulphuric acid because of its low cost, its high relative stability, and the degree to which its rate of reactivity can be modified by changing the temperature. The etchant preferred in the practice of this invention is sulfuric acid in a concentration of 6.5%  $\text{H}_2\text{SO}_4$  by weight in water, and a temperature of 158° F. It should be recognized that although these are the preferred conditions they are not limitations of the invention.

Although the specific example above is a rimmed steel the invention is applicable to killed and semi-killed steels.

We claim:

1. An iron base alloy containing:

|                     | Percent   |
|---------------------|-----------|
| Carbon, maximum     | .010      |
| Manganese           | .15/.75   |
| Molybdenum, maximum | .049      |
| Copper              | .014/.060 |
| Tin                 | .001/.030 |

by weight, the molybdenum, copper and tin in said alloy being in the relationship expressed by the equation

$$(.00489/\text{percent Cu}) - (6.605 \times \text{percent Mo}) - (.084 \times \log_{10} \text{percent Sn}) - (.1367) = X$$

where X is a number between .14 and .46, the balance of said alloy consisting essentially of iron.

2. An iron base alloy being comprised of:

|                 | Percent   | 5 | 2,771,651 | 10/1955 | Morgan  | 75-123 X |
|-----------------|-----------|---|-----------|---------|---------|----------|
| Carbon, maximum | .010      |   | 2,772,154 | 7/1956  | Morgan  | 75-123   |
| Manganese       | .15/.75   |   | 3,183,078 | 5/1965  | Ohtare  | 75-123 X |
| Molybdenum      | .001/.005 |   | 3,193,417 | 6/1965  | Kopchar | 75-123 X |
| Copper          | .014/.040 |   |           |         |         |          |
| Tin             | .001/.005 |   |           |         |         |          |

by weight, the balance of said alloy being essentially iron. 10 P. WEINSTEIN, *Assistant Examiner.*

**References Cited by the Examiner**

UNITED STATES PATENTS

DAVID L. RECK, *Primary Examiner.*